# EUROPEAN PATENT SPECIFICATION

(11) **EP 4 163 411 B1**
(45) Date of publication and mention of the grant of the patent: **05.08.2026**
(21) Application number: 20940134.8
(22) Date of filing: 15.10.2020
(51) Int. Cl.: C23C 2/06, C23C 2/26, C22C 18/00, C23C 30/00, C22C 18/04

(54) **MANUFACTURING METHOD OF A HOT-DIPPED ZINC-ALUMINUM-MAGNESIUM COATED STEEL SHEET**
VERFAHREN ZUR HERSTELLUNG EINES FEUERVERZINKTEN ZINK-ALUMINIUM-MAGNESIUM-BESCHICHTETEN STAHLBLECHS
PROCÉDÉ DE FABRICATION D'UNE TÔLE D'ACIER REVÊTUE D'UN ALLIAGE ZINC-ALUMINIUM-MAGNÉSIUM PAR TREMPAGE À CHAUD

(30) Priority: 08.06.2020 CN 202010513855
(43) Date of publication of application: 12.04.2023
(73) Proprietor: Shougang Group Co., Ltd., Beijing 100041 (CN); Shougang Jingtang Iron & Steel Co., Ltd., Tangshan, Hebei 063200 (CN)
(72) Inventor: JIANG, Guangrui, Beijing 100041 (CN); WANG, Baoyong, Tangshan, Hebei 063200 (CN); LI, Yan, Beijing 100041 (CN); LIU, Datao, Tangshan, Hebei 063200 (CN); TENG, Huaxiang, Beijing 100041 (CN); XU, Chengliang, Beijing 100041 (CN); WANG, Haiquan, Beijing 100041 (CN)
(74) Representative: Valet Patent Services Limited
(86) International application number: PCT/CN2020/121167
(87) International publication number: WO 2021/248765

(56) References cited:
- EP-A1- 3 239 346
- CN-A- 1 398 304
- CN-A- 1 398 304
- CN-A- 105 671 469
- CN-A- 110 004 389
- CN-A- 110 835 757
- CN-A- 110 983 224
- CN-A- 110 983 224
- CN-A- 111 534 777
- TW-A- 201 114 946

## Description

### CROSS-REFERENCE TO RELATED APPLICATIONS

The present disclosure claims the priority to Chinese patent application No. CN202010513855.X, filed on June 8, 2020, entitled "HOT-DIPPED ZINC-ALUMINUM-MAGNESIUM COATED STEEL SHEET WITH EXCELLENT INCISION CORROSION RESISTANCE AND MANUFACTURING METHOD THEREFOR"

### TECHNICAL FIELD

The present disclosure relates to the technical field of steel manufacturing, in particular to a hot-dipped zinc-aluminum-magnesium coated steel sheet and manufacturing method therefor.

### BACKGROUND

Hot-dip galvanizing involves a reaction of molten zinc and alloys thereof with a steel substrate to form a strong metallurgically bonded coating. Such hot-dip galvanized steel has the advantages of strong coating adhesion, long service life, simple manufacturing process, and low product price, and is increasingly in demand in various industries such as the automobile industry, electrical industry and construction industry. The known coated steel sheet is disclosed, e.g., in EP3239346A1, CN1398304A, CN105671469A, and CN110983224A.

Common hot-dip galvanized hot-rolled steel sheet comprises a zinc-only coating. With the increase in corrosion resistance requirement for the hot-dip galvanized hot-rolled steel sheet, the conventional zinc-coated steel sheet has been unable to meet the requirement for the corrosion resistance. Therefore, a hot-dipped zinc-aluminum-magnesium alloy coated steel sheet has been developed.

Although the zinc-aluminum-magnesium alloy coating has good corrosion resistance, it is found in use that when the thickness of the steel sheet is thick, corrosion is likely to occur at the incision position of the steel sheet, which is difficult to meet the needs of use. In addition, in some harsh working environments, the incision position is prone to rust, so an optimized design of the product is required.

Therefore, how to develop a hot-dipped zinc-aluminum-magnesium coated steel sheet with incision corrosion resistance has become an urgent technical problem to be solved.

### SUMMARY

In order to overcome the defect in the prior art, the present disclosure provides a manufacturing method of a hot dipped zinc-aluminium-magnesium coated steel sheet with incision corrosion resistance. The manufacturing method of the hot-dipped zinc-aluminum-magnesium coated steel sheet with incision corrosion resistance provided by the present invention is beneficial for the steel sheet forming a liquid film containing magnesium ion, aluminum ion and zinc ion with good fluidity on the surface in the early stage of atmospheric corrosion, such that the liquid film can fully cover the steel sheet at the incision position and a dense double-layer of hydroxide compound is formed, thereby obtaining the hot-dipped zinc-aluminum-magnesium coated steel sheet with excellent incision corrosion resistance. The present invention is set out in the appended set of claims

In the methods of present invention, a hot-dipped zinc-aluminum-magnesium coated steel sheet is provided, which may include a steel sheet and a coating, characterized in that, mass fractions of chemical components in the coating are: 2%~12% for aluminum, 1%~4% for magnesium, and rest being zinc and inevitable impurities; the mass fraction of aluminum is 2 to 3 times the mass fraction of magnesium; and a thickness of the coating is not less than 5‰ of a thickness of the steel sheet.

The mass fraction of aluminum is 2 to 3 times the mass fraction of magnesium.

The thickness of the steel sheet may range from 0.5 mm to 6 mm.

In an alternative method according to claim 2, the mass fractions of magnesium and aluminum in the coating may be controlled based on the thickness of the steel sheet, specifically including: when 0.5 mm ≤ the thickness of the steel sheet ≤ 2 mm, the mass fractions of the chemical components in the coating may be: 2% ~ 12% for aluminum, 1% ~ 4% for magnesium, and the rest being zinc and inevitable impurities; when 2 mm < the thickness of the steel sheet ≤ 4 mm, the mass fractions of the chemical components in the coating may be: 3% ~ 12% for aluminum, 1.5% ~4% for magnesium, and the rest being zinc and inevitable impurities; when 4 mm < the thickness of the steel sheet ≤ 5 mm, the mass fractions of the chemical components in the coating may be: 4% ~ 12% for aluminum, 2% ~ 4% for magnesium, and the rest being zinc and inevitable impurities; and when 5 mm < the thickness of the magnesium, 0.01% ~ 0.1% for calcium, and rest being zinc and inevitable impurities; the mass fraction of aluminum may be 2 to 3 times the mass fraction of magnesium; and a thickness of the coating may be not less than 5‰ of a thickness of the steel sheet.

In the method of claim 2, when the mass fraction of calcium is 0.01%, the mass fractions of magnesium and aluminum in the coating may be controlled based on the thickness of the steel sheet, specifically including: when 0.5 mm ≤ the thickness of the steel sheet ≤ 2.5 mm, the mass fractions of the chemical components in the coating may be: 2% ~ 12% for aluminum, 1% ~ 4% for magnesium, and the rest being zinc and inevitable impurities; when 2.5 mm < the thickness of the steel sheet ≤ 4 mm, the mass fractions of the chemical components in the coating may be: 2.5% ~ 12% for aluminum, 1.2% ~ 4% for magnesium, and the rest being zinc and inevitable impurities; when 4 mm < the thickness of the steel sheet ≤ 5 mm, the mass fractions of the chemical components in the coating may be: 3.8% ~ 12% for aluminum, 1.8% ~ 4% for magnesium, and the rest being zinc and inevitable impurities; and when 5 mm < the thickness of the steel sheet ≤ 6 mm, the mass fractions of the chemical components in the coating may be: 5% ~ 12% of aluminum, 2.5% ~ 4% for magnesium, and the rest being zinc and inevitable impurities.

A manufacture method of a hot-dipped zinc-aluminum-magnesium coated steel sheet with incision corrosion resistance according to claims 1 or 2 is provided, characterized in that, the manufacture method includes:
obtaining a coating solution by using chemical components of a coating of the hot-dipped zinc-aluminum-magnesium coated steel sheet with incision corrosion resistance; heating the coating solution to obtain a preheated coating solution with a temperature of the preheated coating solution being controlled to be not lower than a melting point of the coating solution and not higher than 500°C; obtaining a steel sheet and immersing the steel sheet in the preheated coating solution to obtain a coated steel sheet; and cooling the coated steel sheet to obtain the hot-dipped zinc-aluminum-magnesium coated steel sheet with incision corrosion resistance.

In the inventive methods, the cooling the coated steel sheet may include: when a temperature of the coated steel sheet is between a temperature of the coating bath and 360°C, cooling may be performed at a first cooling rate and the first cooling rate may be controlled at: 0 < the first cooling rate ≤ 1°C/s; when the temperature of the coated steel sheet is between 360°C and 300°C, cooling may be performed at a second cooling rate and the second cooling rate may be ≥ 5°C/s.

In some embodiments, the cooling the coated steel sheet may include: blowing air or spraying water on the surface of the coating of the coated steel sheet for cooling.

In some embodiments, the steel sheet may be preheated to a steel sheet preheating temperature before the immersion of the steel sheet in the coating solution for bathing. The range of the steel sheet preheating temperature is the temperature of the preheated coating solution ± 10°C.

In some embodiments, the steel sheet may be preheated to the steel sheet preheating temperature before the immersion of the steel sheet in the coating solution for bathing, and the steel sheet preheating temperature is controlled based on the thickness of the steel sheet, specifically including: when 0.5 mm ≤ the thickness of the steel sheet ≤ 2 mm, the temperature of the preheated coating solution ≤ the steel sheet preheating temperature ≤ the temperature of the preheated coating solution + 10°C; when 2 mm < the thickness of the steel sheet ≤ 4 mm, the temperature of the preheated coating solution - 5°C ≤ the steel sheet preheating temperature ≤ the temperature of the preheated coating solution; when 4 mm < the thickness of the steel sheet ≤ 6 mm, the temperature of the preheated coating solution - 10°C ≤ the steel sheet preheating temperature ≤ the temperature of the preheated coating solution - 5°C.

In some embodiments, the obtaining the steel sheet may include: obtaining the steel sheet with a surface roughness Ra of 1 µm ~ 2 µm.

One or more technical solutions according to the embodiments of the present disclosure have at least the following technical effects or advantages: the hot-dipped zinc-aluminum-magnesium coated steel sheet with incision corrosion resistance and the manufacturing method thereof provided by the present disclosure include: (1) in terms of chemical components, 2% ~ 12% for aluminum, 1% ~ 4% for magnesium, and the rest being zinc and inevitable impurities, wherein the content of aluminum in mass fraction is 2 to 3 times that of magnesium and the thickness of the coating is not less than 5‰ of the thickness of the steel sheet; and (2) in terms of process, the temperature of the preheated coating solution is controlled to be not lower than the melting point of the coating solution and not higher than 500°C, which is beneficial for the steel sheet forming the liquid film containing magnesium ion, aluminum ion and zinc ion with good fluidity on the surface in the early stage of atmospheric corrosion, such that the liquid film can fully cover the steel sheet at the incision position and a dense double-layer of hydroxide compound is formed, thereby obtaining the hot-dipped zinc-aluminum-magnesium coated steel sheet with excellent incision corrosion resistance.

### BRIEF DESCRIPTION OF THE DRAWINGS

In order to illustrate the technical solutions in the embodiments of the present disclosure more clearly, the following briefly introduces the accompanying drawings used in the description of the embodiments. Obviously, the accompanying drawings in the following description are some examples of the present disclosure.
FIG. 1 is a flow chart illustrating the protection of an incision by a zinc-aluminum-magnesium coating according to an embodiment of the present disclosure.
FIG. 2 is a flow chart illustrating the manufacturing method of the hot-dipped zinc-aluminum-magnesium coated steel sheet according to the present disclosure

### DETAILED DESCRIPTIONN

The present disclosure will be described in detail below with reference to specific embodiments and examples, and the advantages and various effects of the present disclosure will be more clearly presented therefrom.

The terms used throughout the specification are to be understood as commonly used in the art, unless specifically stated otherwise. Therefore, unless otherwise defined, all technical and scientific terms used herein have the same meaning as commonly understood by one of ordinary skill in the art to which the present disclosure belongs. In case of conflict, the present specification takes precedence.

Unless otherwise specified, various raw materials, reagents, instruments and equipment, etc. used in the present disclosure are commercially available or can be obtained by existing methods.

An embodiment of the present invention provides a hot-dipped zinc-aluminum-magnesium coated steel sheet with incision corrosion resistance, the general idea of which is as follows.

In order to overcome the defect in the prior art, an embodiment of the present disclosure provides a hot-dipped zinc-aluminum-magnesium coated steel sheet with incision corrosion resistance, which may include a steel sheet and a coating; a mass percentage of chemical components in the coating may be: 2% ~ 12% for aluminum, 1% ~ 4% for magnesium, and rest being zinc and inevitable impurities; the content of aluminum in mass fraction may be 2 to 3 times that of magnesium; and a thickness of the coating may be not less than 5‰ of a thickness of the steel sheet.

In some embodiments of the present disclosure, FIG. 1 illustrates a flow chart of incision protection by a zinc-aluminum-magnesium coating. In the early stage of atmospheric corrosion, water vapor in the atmosphere condenses on the surface of the coating to form a water film; the magnesium element in the coating first undergoes an anodic corrosion reaction and form magnesium ions, which are dissolved in the water film; and the magnesium ions combine with hydroxide and carbonate groups formed by a cathodic reaction to form compounds such as magnesium carbonate and basic magnesium carbonate with good fluidity. In addition, the aluminum and zinc in the coating also undergo the anodic corrosion reaction to form aluminum ions and zinc ions dissolved in the liquid film. These compounds containing magnesium ions and aluminum ions flow with the liquid film to the incision position of the steel sheet. Due to the presence of magnesium ions and aluminum ions, the pH value in the liquid film will not exceed 10, so that zinc ions will not form loose and porous zinc oxide, but tend to form dense oxides such as basic zinc carbonate and basic zinc chloride. These compounds, in turn, form a dense protective hydroxide double-layer with magnesium carbonate and aluminum hydroxide, etc., which provides a good protective effect on the incision. However, in order for the incision position of the steel sheet to be covered by these protective layers, it is required to the steel sheet form a liquid film containing magnesium ion, aluminum ion and zinc ion with good fluidity on the surface in the early stage of atmospheric corrosion, such that the liquid film can fully cover the steel sheet at the incision position and a dense double-layer of hydroxide compound is formed.

In some embodiments of the present disclosure, the reason why the mass fraction of magnesium can be set as 1% ~ 4% is that: first, a certain amount of magnesium is required in the coating and the main function of magnesium is to make the steel sheet form an aqueous solution or a liquid film with good fluidity on the surface in the early stage of atmospheric corrosion. On the one hand, this aqueous solution or the liquid film containing magnesium ions can accelerate the dissolution of aluminum and zinc to form aluminum ions and zinc ions; on the other hand, it prevents aluminum ions and zinc ions in solution from rapidly precipitating into loose compounds, instead, the solution containing the aluminum ion and zinc ion is allowed to react slowly with carbon dioxide and the like in the atmosphere to form dense oxides. If the magnesium content in the coating layer is less than 1%, this effect cannot be exhibited. However, if the magnesium content is too high, it is easy to form too thick magnesium oxide on the surface, which is not conducive to the dissolution of aluminum and zinc. At the same time, it is easy to form Mg-Zn compound hard particles that are embedded in the coating and cause electrochemical corrosion effect and thus reduce the corrosion resistance of the coating. Therefore, the magnesium content should not exceed 4%.

In some embodiments of the present disclosure, the reason why the mass fraction of aluminum can be set as 2% ~ 12% is that: the content of aluminum in the coating layer should not be less than 2%, since aluminum is the main framework element for forming the bilayer compound and is also the main element that fills the voids of loose zinc oxide and zinc hydroxide. If the aluminum content is too high, it will cause a severe galvanic corrosion effect, and a corrosion current will be formed between aluminum and zinc, which reduces the corrosion resistance of the coating. The maximum aluminum content in the coating is 12%.

In some embodiments of the present disclosure, the reason why the content of aluminum in mass fraction may be 2 to 3 times the mass fraction of magnesium is that: in the early stage of atmospheric corrosion, the water vapor in the atmosphere condenses into the surface of the coating and form a water film. The magnesium element in the coating first undergoes an anodic reaction to form magnesium ions dissolved in the water film, and the magnesium ions combine with the hydroxide and carbonate formed by the cathodic reaction to produce basic magnesium carbonate Mg(OH)₂ • MgCO₃ and magnesium hydroxide Mg(OH)₂. Due to the presence of magnesium ions and aluminum ions, the pH value in the water film will not exceed 10, so that zinc ions will not form loose and porous zinc oxide, but tend to form dense oxides such as basic zinc carbonate and basic zinc chloride. These compounds, in turn, form a dense protective hydroxide double-layer with magnesium carbonate and aluminum hydroxide, etc., which provides a good protective effect on the incision. This protective hydroxide double-layer (LDH) comprises MgAl-LDH and ZnAl-LDH, wherein the numbers of Mg atom and Al atom in the former molecule is 6 and 2, respectively, and the number of Al atom in the latter molecule is 2. In terms of stability, the stability of ZnAl-LDH is more than 5 times that of MgAl-LDH, so generally it is the formation of ZnAl-LDH hydroxide double-layer that protects the coating and incision and improves the corrosion resistance. When the total amount of ZnAl-LDH is 5 times that of MgAl-LDH, the total content of Al in the hydroxide double-layer is 2 times that of Mg. Therefore, the content of Al in the coating is at least 2 times that of Mg. However, if there are too many aluminum ions in the coating, excess Al(OH)₄⁻ compound will be easily precipitated in the early stage, which prevents the formation of a dense hydroxide double-layer. In some embodiments of the present disclosure, the content of aluminum in the coating is preferably 2.3 times the content of magnesium, so that the oxidation of magnesium can be significantly inhibited.

In some embodiments of the present disclosure, the reason why the thickness of the coating may not be less than 5‰ of the thickness of the steel sheet is that: if the thickness of the coating is less than 5‰ of the thickness of the steel sheet, the protective compound double-layer cannot cover sides of the incision of the steel sheet and thus is also impossible to protect the incision of the steel sheet.

In the present invention, the mass fraction of chemical components in the coating may be: 2% ~ 12% for aluminum, 1% ~ 4% for magnesium, and the rest being zinc and inevitable impurities, wherein the content of aluminum in mass fraction may be 2 to 3 times the content of magnesium and the thickness of the coating may be not less than 5‰ of the thickness of the steel sheet, which together facilitate the formation of the liquid film containing magnesium ion, aluminum ion and zinc ion with good fluidity on the coating in the early stage of atmospheric corrosion and are beneficial for the liquid film to fully cover the steel sheet at the incision position and to form a dense double-layer of hydroxide compound, thereby obtaining the hot-dipped zinc-aluminum-magnesium coated steel sheet with excellent incision corrosion resistance.

In the present invention, the thickness of the steel sheet may range from 0.5 mm to 6 mm. In the case of relying on the zinc-aluminum-magnesium coating to protect the incision of the steel sheet, there are certain requirements for the thickness of the steel sheet. If the steel sheet is too thick, excellent incision corrosion resistance cannot be achieved. The thickness should generally not exceed 6 mm. If the steel sheet is too thin, there is also a certain risk for application, since the too-thin incision will form extremely sharp corners and pits from the microscopic point of view. The radius of curvature at these locations is often less than the minimum radius of curvature that can be wetted by the surface tension of an aqueous solution. Therefore, they cannot be covered with the solution containing aluminum ions and magnesium ions, so that a protective layer cannot be formed. In some embodiments of the present disclosure, the thickness of the steel sheet is required to be no less than 0.5 mm.

The applicant has found through research that the thicker the steel sheet, the higher the content of aluminum and magnesium required to achieve better incision corrosion resistance. Specifically: when the thickness of the steel sheet is no more than 2 mm, having the magnesium content being 1% and the aluminum content being 2% in the coating can provide a good incision protection effect, of course, the premise is that the manufacturing requirements of the present disclosure are met. However, as the thickness of the steel sheet increases, lower limits of the required aluminum content and the required magnesium content increase accordingly. Generally, when the thickness of the steel sheet reaches 4 mm, the magnesium content in the coating should not be less than 1.5% and the aluminum content in the coating should not be less than 3%; when the thickness of the steel sheet reaches 5 mm, the magnesium content in the coating should not be less than 2% and the aluminum content in the coating should not be less than 4%; and when the thickness of the steel sheet reaches 6 mm, the magnesium content in the coating should not be less than 3% and the aluminum content in the coating should not be less than 6%.

The applicant further found through research that adding a certain amount of Ca element to the coating can inhibit the formation of large particles of Mg-Zn compounds on the surface, prevent the premature reaction of aluminum and hydroxide to form precipitation, and improve the fluidity of aluminum ions, so that magnesium ions and aluminum ions are able to more adequately cover the incision site. Therefore, adding a certain amount of Ca element to the coating can improve the corrosion resistance of the incision. In some embodiments of the present disclosure, the addition amount of Ca element may exceed 0.01%, and the Mg-Zn compound formed therefrom changes from polygonal particles to blunt round particles, and the particle size can be further reduced from 50 microns to no more than 20 microns. If the addition of Ca element exceeds 0.1%, it is easy to cause zinc dross defects in production and produce galvanic corrosion, thereby reducing the corrosion resistance of the coating. In some embodiments of the present disclosure, the addition amount of calcium element may be 0.01% to 0.1%, and it should also satisfy: 2% ~ 12% for aluminum, 1% ~ 4% for magnesium, and the rest being zinc and inevitable impurities; the content of aluminum in mass fraction may be 2 to 3 times that of magnesium; and the thickness of the coating may be not less than 5‰ of that of the steel sheet.

In the present invention, in the case of adding 0.01% Ca, when the thickness of the steel sheet does not exceed 2.5 mm, the magnesium content in the coating can be 1%, and the aluminum content in the coating can be 2%, such that the coating can provide good incision protection effect. In some embodiments of the present disclosure, when the thickness of the steel sheet reaches 4 mm, the magnesium content in the coating should not be less than 1.2% and the aluminum content in the coating should not be less than 2.5%; when the thickness of the steel sheet reaches 5 mm, the magnesium content in the coating should not be less than 1.8% and the aluminum content in the coating should not be less than 3.8%; and when the thickness of the steel sheet reaches 6 mm, the magnesium content in the coating should not be less than 2.5% and the aluminum content in the coating should not be less than 5%.

The present invention provides a manufacture method of a hot-dipped zinc-aluminum-magnesium coated steel sheet with incision corrosion resistance according to the appended claims, which may include: obtaining a coating solution by using chemical components of a coating of the hot-dipped zinc-aluminum-magnesium coated steel sheet with incision corrosion resistance; heating the coating solution to obtain a preheated coating solution with a temperature of the preheated coating solution being controlled to be not lower than a melting point of the coating solution and not higher than 500°C; obtaining a steel sheet, and immersing the steel sheet in the preheated coating solution to obtain a coated steel sheet; and cooling the coated steel sheet to obtain the hot-dipped zinc-aluminum-magnesium coated steel sheet with incision corrosion resistance.

The temperature of the preheated coating solution may be controlled to be not lower than the melting point of the coating solution and not higher than 500°C. The reason is: if the temperature of the preheated coating solution is too high, the oxidation reaction in the coating bath is violent and the alloying elements on the surface of the coating bath are easily oxidized and evaporated, so that the distribution of the alloying elements in the coating bath is uneven. There are few elements in the surface layer but more elements in the inner layer. Such a nonuniform distribution of the elements in the coating will greatly deteriorate the corrosion resistance of the coating. In some embodiments of the present disclosure, the temperature of the preheated coating solution cannot exceed 500°C. On the other hand, if the temperature of the preheated coating solution is lower than the melting point of the coating solution, the coating solution will solidify.

In some embodiments of the present disclosure, the obtained steel sheet may have a surface roughness Ra of 1 µm ~ 2 µm. The rough surface morphology of the steel sheet is conducive to improving the adhesion between the coating and the steel sheet, improving the corrosion resistance of the coating during the corrosion process, and making the coating not easily peeled off. But if the surface of the steel sheet is too rough, the following adverse effects will occur: parts of the coating will be significantly thinned and the corrosion resistance of the coating will decrease; the rough ridge on the steel sheet will react rapidly during hot-dipping, forming an excessively thick Fe-Al-Zn compound layer, which consumes aluminum in the coating solution, so that the corrosion resistance of the coating will decrease due to insufficient aluminum in the local area of the coating. Therefore, in some embodiments of the present disclosure, the surface roughness Ra of the obtained steel sheet may be limited to not more than 2.0 µm and not less than 1.0 µm.

In some embodiments of the present disclosure, the steel sheet may be preheated to a steel sheet preheating temperature before the immersion of the steel sheet in the coating solution for bathing, and the steel sheet preheating temperature is controlled according to the thickness of the steel sheet, specifically including: when 0.5 mm ≤ the thickness of the steel sheet ≤ 2 mm, the temperature of the preheated coating solution ≤ the steel sheet preheating temperature ≤ the temperature of the preheated coating solution + 10°C; when 2 mm < the thickness of the steel sheet ≤ 4 mm, the temperature of the preheated coating solution - 5°C ≤ the steel sheet preheating temperature ≤ the temperature of the preheated coating solution; and when 4 mm < the thickness of the steel sheet ≤ 6 mm, the temperature of the preheated coating solution - 10°C ≤ the steel sheet preheating temperature ≤ the temperature of the preheated coating solution - 5°C.

In some embodiments of the present disclosure, when 0.5 mm ≤ the thickness of the steel sheet ≤ 2 mm, before hot-dipping, the steel sheet preheating temperature may range from the temperature of the preheated coating solution to a temperature 10°C higher than the temperature of the preheated coating solution (i.e., the temperature of the preheated coating solution ≤ the steel sheet preheating temperature ≤ the temperature of the preheated coating solution + 10°C). This is to ensure the formation of a stable Fe-Al-Zn compound between the steel sheet and the coating solution, improve the adhesion of the coating, and make the coating not easily peeled off. However, if the temperature is too high, the compound will be too thick, resulting in loss of corrosion resistance due to the reduction of aluminum in the coating. If the thickness of the steel sheet exceeds 2 mm, during the reaction between the steel sheet and the coating solution, the temperature inside the steel sheet cannot be lowered in time and thus the heat cannot be conducted out in time. When the temperature of the steel sheet is too high, the heat inside the steel sheet will continue to flow to the outside of the surface of the steel sheet, making the Fe-Al-Zn compound layer formed between the steel sheet and the coating solution too thick, which consumes the aluminum in the coating solution instead, resulting in the loss of corrosion resistance due to the reduction of aluminum in the coating layer. Therefore, in some embodiments of the present disclosure, when the thickness of the steel sheet exceeds 2 mm but does not exceed 4 mm, the steel sheet preheating temperature may range from a temperature 5°C lower than the temperature of the preheated coating solution to the temperature of the preheated coating solution (i.e., the temperature of preheated coating solution - 5°C ≤ the steel sheet preheating temperature ≤ the temperature of the preheated coating solution); and in some embodiments of the present disclosure, when the thickness of the steel sheet exceeds 4 mm but does not exceed 6 mm, the steel sheet preheating temperature may range from a temperature 10°C lower than the temperature of the preheated coating solution to a temperature 5°C lower than the temperature of the preheated solution (i.e., the temperature of the preheated coating solution - 10°C ≤ the steel sheet preheating temperature ≤ the temperature of the preheated coating solution - 5°C).

In some embodiments of the present disclosure, the cooling the coated steel sheet may include: blowing air or spraying water on a surface of the coating of the coated steel sheet for cooling.

In the present invention, the cooling includes a two-stage cooling, specifically: when the temperature of the coated steel sheet is between the temperature of the coating bath and 360°C, cooling may be performed at a first cooling rate and the first cooling rate may be controlled at: 0 < the first cooling rate ≤ 1°C/s; when the temperature of the coated steel sheet is between 360°C and 300°C, cooling may be performed at a second cooling rate and the second cooling rate may be > 5°C/s. The inventors found that when the coating begins to solidify, the coating solution and the substrate rapidly react and form an aluminum-rich compound, and at the same time, a large precipitation of aluminum-rich crystals is formed first. If the cooling rate is appropriate, the formation of a large number of dendrites rich in aluminum and magnesium is favored. Such dendrites rich in aluminum and magnesium are difficult to react with media in subsequent corrosion process and thus have good corrosion resistance. The inventors have also found that when the temperature of the coating is lowered to below 360°C, all the crystals that precipitate first have been all precipitated, and a eutectic reaction process begins. During the eutectic reaction, a mixture structure containing one or more of Al/Zn/Mg-Zn, Al/Mg-Zn or Zn/Mg-Zn is formed. The mixture structure is in different phases and is fine and dense. In subsequent use, such fine and dense mixture structure can quickly react with carbon dioxide and water in the air to form an aqueous solution containing zinc, aluminum and magnesium, which can cover and protect the incision. Therefore, in some embodiments of the present disclosure, in order to form a large amount of dendrites rich in aluminum and magnesium, when the temperature of the coated steel sheet is between the temperature of the coating bath and 360°C, cooling may be performed at the first cooling rate and the first cooling rate may be controlled at: 0 < the first cooling rate ≤ 1°C/s. In some embodiments of the present disclosure, in order to promote the formation of a fine and dense eutectic structure (a mixture structure containing one or more of Al/Zn/Mg-Zn, Al/Mg-Zn or Zn/Mg-Zn) on the surface of the coating, when the temperature of the coated steel sheet is between 360°C and 300°C, cooling may be performed at the second cooling rate and the second cooling rate may be ≥ 5°C/s.

One or more technical solutions of the embodiments of the present disclosure are beneficial for the steel sheet forming the liquid film containing magnesium ion, aluminum ion and zinc ion with good fluidity on the surface in the early stage of atmospheric corrosion, such that the liquid film can fully cover the steel sheet at the incision position and a dense double-layer of hydroxide compound is formed, thereby obtaining a hot-dipped zinc-aluminum-magnesium coated steel sheet with excellent incision corrosion resistance.

A hot-dipped zinc-aluminum-magnesium coated steel sheet with incision corrosion resistance and manufacturing method therefor of the present disclosure are described in detail below in combination with experimental data. A hot-rolled steel sheet was used as the substrate, and the material of the hot-rolled steel sheet was CQ grade.

Test groups 1-17 were established according to one or more technical solutions of the embodiments of the present disclosure. In addition, comparison groups 1-12 were established. Among them, the test groups 1-6 and the comparison groups 1-6 use cold-rolled steel sheet as the substrate, and the material of the steel sheet was CQ grade. The test groups 7-17 and the comparison groups 7-12 use the hot-rolled steel sheet as the substrate, and the material of the steel sheet was CQ grade. In the test groups 1-17 and the comparative groups 1-12, the coated steel sheet was prepared according to the relevant steps in the manufacturing method of the hot-dipped zinc-aluminum-magnesium coated steel sheet with incision corrosion resistance provided by the present disclosure. The difference among the test groups 1-17 and the comparison groups 1-12 was the chemical compositions of the coating solutions as shown in Table 1. Specific manufacturing processes and parameters are shown in Table 2.

**Table 1**

| Group | Al content in coating | Mg content in coating | Ca content in coating | Al content/Mg content in coating | Thickness of coating | Thickness of steel sheet | Thickness of coating/Thic kness of steel sheet |
|---|---|---|---|---|---|---|---|
| | wt% | wt% | wt% | | micro | mm | |
| Test group 1 | 2 | 1 | 0 | 2.0 | 5 | 0.5 | 1.00% |
| Test group 2 | 2.5 | 1 | 0 | 2.5 | 7 | 1 | 0.70% |
| Test group 3 | 3 | 1.5 | 0 | 2.0 | 10 | 1.5 | 0.67% |
| Test group 4 | 4 | 1.5 | 0.1 | 2.7 | 20 | 2.5 | 0.80% |
| Test group 5 | 3.8 | 1.5 | 0.01 | 2.5 | 20 | 3 | 0.67% |
| Test group 6 | 2.5 | 1.0 | 0.05 | 2.5 | 15 | 2.8 | 0.54% |
| Test group 7 | 6 | 3 | 0 | 2.0 | 30 | 6 | 0.50% |
| Test group 8 | 4.5 | 2 | 0 | 2.3 | 30 | 5 | 0.60% |
| Test group 9 | 8 | 3.5 | 0 | 2.3 | 40 | 4 | 1.00% |
| Test group 10 | 11 | 4 | 0 | 2.8 | 20 | 4 | 0.50% |
| Test group 11 | 12 | 4 | 0 | 3.0 | 30 | 5 | 0.60% |
| Test group 12 | 9 | 3.2 | 0.05 | 2.8 | 30 | 6 | 0.50% |
| Test group 13 | 2.4 | 1 | 0.01 | 2.4 | 30 | 3 | 1.00% |
| Test group 14 | 2.5 | 1.2 | 0.02 | 2.1 | 30 | 4 | 0.75% |
| Test group 15 | 3.8 | 1.5 | 0.05 | 2.5 | 30 | 5 | 0.60% |
| Test group 16 | 6 | 2 | 0.02 | 3.0 | 30 | 5 | 0.60% |
| Test group 17 | 5 | 2.5 | 0.08 | 2.0 | 30 | 6 | 0.50% |
| Comparison group 1 | 1.2 | 1 | 0 | 1.2 | 8 | 1 | 0.80% |
| Comparison group 2 | 3 | 0.5 | 0 | 6.0 | 10 | 1.2 | 0.83% |
| Comparison group 3 | 3 | 2 | 0 | 1.5 | 7 | 1.2 | 0.58% |
| Comparison group 4 | 4 | 2 | 0.2 | 2.0 | 5 | 2 | 0.25% |
| Comparison group 5 | 5 | 3 | 0 | 1.7 | 4 | 0.25 | 1.60% |
| Comparison group 6 | 2 | 2 | 0 | 1.0 | 10 | 2.5 | 0.40% |
| Comparison group 7 | 3 | 5 | 0 | 0.6 | 8 | 4 | 0.20% |
| Comparison group 8 | 15 | 6 | 0.2 | 2.5 | 20 | 5 | 0.40% |
| Comparison group 9 | 13 | 2 | 0.01 | 6.5 | 7 | 5 | 0.14% |
| Comparison group 10 | 4 | 2 | 0 | 2.0 | 40 | 6 | 0.67% |
| Comparison group 11 | 6 | 3 | 0 | 2.0 | 40 | 8 | 0.50% |
| Comparison group 12 | 8 | 2 | 0 | 4.0 | 30 | 8 | 0.38% |

**Table 2**

| Group | Temperature of preheated coating solution | Temperature of preheated steel sheet | Roughness of steel sheet | First cooling rate | Second cooling rate |
|---|---|---|---|---|---|
| | °C | °C | micro | °C/s | °C/s |
| Test group 1 | 420 | 420 | 1 | 0.5 | 10 |
| Test group 2 | 440 | 440 | 1.2 | 0.1 | 12 |
| Test group 3 | 430 | 430 | 1.3 | 0.4 | 12 |
| Test group 4 | 450 | 445 | 1.5 | 0.2 | 10 |
| Test group 5 | 500 | 495 | 1.9 | 0.8 | 5 |
| Test group 6 | 410 | 408 | 2 | 1 | 8 |
| Test group 7 | 440 | 430 | 2 | 0.1 | 10 |
| Test group 8 | 450 | 445 | 1.2 | 0.2 | 12 |
| Test group 9 | 490 | 487 | 1.9 | 0.9 | 12 |
| Test group 10 | 500 | 496 | 1.9 | 0.3 | 10 |
| Test group 11 | 400 | 390 | 1 | 0.9 | 5 |
| Test group 12 | 400 | 393 | 2 | 0.9 | 8 |
| Test group 13 | 450 | 445 | 1.3 | 0.1 | 12 |
| Test group 14 | 430 | 420 | 1.2 | 0.2 | 5 |
| Test group 15 | 430 | 420 | 1.8 | 0.2 | 11 |
| Test group 16 | 450 | 440 | 1.9 | 0.8 | 10 |
| Test group 17 | 450 | 440 | 2 | 0.03 | 8 |
| Comparison group 1 | 460 | 460 | 0.8 | 1.2 | 3 |
| Comparison group 2 | 470 | 480 | 0.8 | 0.3 | 8 |
| Comparison group 3 | 430 | 450 | 1.2 | 3 | 10 |
| Comparison group 4 | 510 | 510 | 1.2 | 0.4 | 12 |
| Comparison group 5 | 520 | 500 | 1.5 | 0.8 | 12 |
| Comparison group 6 | 430 | 440 | 2.1 | 0.2 | 2 |
| Comparison group 7 | 500 | 460 | 2.3 | 0.2 | 12 |
| Comparison group 8 | 550 | 500 | 4.3 | 5 | 9 |
| Comparison group 9 | 590 | 500 | 2.1 | 5 | 3 |
| Comparison group 10 | 450 | 450 | 2.9 | 0.2 | 12 |
| Comparison group 11 | 430 | 450 | 1.2 | 0.8 | 12 |
| Comparison group 12 | 470 | 460 | 1.9 | 0.2 | 2 |

The incision corrosion resistance was evaluated for the zinc-aluminum-magnesium coated steel sheets obtained from the above test groups 1-17 and comparative groups 1-12. A neutral salt spray testing was used for evaluation for 480 hours and the area ratio of red rust at the incision position was observed. Using a bending method, the zinc-aluminum-magnesium-coated steel sheets obtained from the test groups 1-17 and the comparison groups 1-12 were respectively bent by 90° and then the proportion of peeling of the coating was observed. The experimental evaluation results are shown in Table 3.

**Table 3**

| Group | Area ratio of red rust (%) | Proportion of peeling of coating (%) |
|---|---|---|
| Test group 1 | 1 | 0 |
| Test group 2 | 3 | 0 |
| Test group 3 | 2 | 0 |
| Test group 4 | 0 | 0 |
| Test group 5 | 0 | 0 |
| Test group 6 | 0 | 0 |
| Test group 7 | 1 | 0 |
| Test group 8 | 3 | 0 |
| Test group 9 | 2 | 0 |
| Test group 10 | 2 | 0 |
| Test group 11 | 2 | 0 |
| Test group 12 | 0 | 0 |
| Test group 13 | 0 | 0 |
| Test group 14 | 0 | 0 |
| Test group 15 | 0 | 0 |
| Test group 16 | 0 | 0 |
| Test group 17 | 0 | 0 |
| Comparison group 1 | 12 | 2 |
| Comparison group 2 | 17 | 2 |
| Comparison group 3 | 15 | 0 |
| Comparison group 4 | 10 | 0 |
| Comparison group 5 | 18 | 0 |
| Comparison group 6 | 20 | 4 |
| Comparison group 7 | 14 | 5 |
| Comparison group 8 | 20 | 10 |
| Comparison group 9 | 21 | 10 |
| Comparison group 10 | 20 | 0 |
| Comparison group 11 | 34 | 0 |
| Comparison group 12 | 23 | 0 |

As can be seen from Table 3, as for the hot-dipped zinc-aluminum-magnesium coated steel sheet with incision corrosion resistance obtained in the test groups 1-17, the area ratios of red rust were in the range of 0 ~ 3%; and the proportions of peeling of the coating were all 0%. As for the hot-dipped zinc-aluminum-magnesium coated steel sheet with incision corrosion resistance obtained in the comparative groups 1-12, the area ratios of red rust were in the range of 12% ~ 34%; and the proportions of peeling of the coating were 2% ~ 10%. Obviously, the hot-dipped zinc-aluminum-magnesium coated steel sheet with incision corrosion resistance obtained according to the test groups 1-17 of the embodiments of the present disclosure showed a significant lower percentage of red rust area and peeling in coating.

In the comparison groups 1-12, the incision corrosion resistance was poor since the coating did not satisfy the following requirements: 2% ~ 12% for aluminum, 1% ~ 4% for magnesium, and the rest being zinc and inevitable impurities; the content of aluminum in mass fraction is 2 to 3 times the content of magnesium; and the thickness of the resulted coating is not less than 5‰ of the thickness of the steel sheet.

To sum up, the manufacturing method of the hot-dipped zinc-aluminum-magnesium coating with incision corrosion resistance provided by the present disclosure is beneficial for the steel sheet forming the liquid film containing magnesium ion, aluminum ion and zinc ion with good fluidity on the surface in the early stage of atmospheric corrosion, such that the liquid film can fully cover the steel sheet at the incision position and a dense double-layer of hydroxide compound is formed, thereby obtaining the hot-dipped zinc-aluminum-magnesium coated steel sheet with excellent incision corrosion resistance.

The scope of the invention and possible modifications are defined by the scope of the appended claims.

## Claims

1. A manufacturing method of a hot-dipped zinc-aluminum-magnesium coated steel sheet with incision corrosion resistance, **characterized in that** the hot-dipped zinc-aluminum-magnesium coated steel sheet comprises a steel sheet and a coating,
mass fractions of chemical components in the coating are: 2% ~ 12% for aluminum, 1% ~ 4% for magnesium, and rest being zinc and inevitable impurities; and the mass fraction of aluminum is 2 to 3 times the mass fraction of magnesium; and
a thickness of the coating is not less than 5‰ of a thickness of the steel sheet;
wherein, the thickness of the steel sheet ranges from 0.5 mm to 6 mm;
wherein the mass fractions of magnesium and aluminum in the coating are controlled based on the thickness of the steel sheet, comprising:
when 0.5 mm ≤ the thickness of the steel sheet ≤ 2 mm, the mass fractions of the chemical components in the coating are: 2% ~ 12% for aluminum, 1% ~ 4% for magnesium, and the rest being zinc and inevitable impurities;
when 2 mm < the thickness of the steel sheet ≤ 4 mm, the mass fractions of the chemical components in the coating are: 3% ~ 12% for aluminum, 1.5% ~ 4% for magnesium, and the rest being zinc and inevitable impurities;
when 4 mm < the thickness of the steel sheet ≤ 5 mm, the mass fractions of the chemical components in the coating are: 4% ~ 12% of aluminum, 2% ~ 4% of magnesium, and the rest being zinc and inevitable impurities; and
when 5 mm < the thickness of the steel sheet ≤ 6 mm, the mass fractions of the chemical components in the coating are: 6% ~ 12% for aluminum, 3% ~ 4% for magnesium, and the rest being zinc and inevitable impurities;
wherein the manufacturing method comprises:
obtaining a coating solution by using the chemical components of the coating of the hot-dipped zinc-aluminum-magnesium coated steel sheet;
heating the coating solution to obtain a preheated coating solution with a temperature of the preheated coating solution being controlled to be not lower than a melting point of the coating solution and not higher than 500°C;
obtaining a steel sheet, and immersing the steel sheet in the preheated coating solution to obtain a coated steel sheet; and
cooling the coated steel sheet to obtain the hot-dipped zinc-aluminum-magnesium coated steel sheet;
wherein the cooling the coated steel sheet comprises:
when a temperature of the coated steel sheet is between a temperature of the coating bath and 360°C, the cooling is performed at a first cooling rate and the first cooling rate is controlled at: 0 < the first cooling rate ≤ 1°C/s; and
when the temperature of the coated steel sheet is between 360°C and 300°C, the cooling is performed at a second cooling rate and the second cooling rate is ≥ 5°C/s.

2. A manufacturing method of a hot-dipped zinc-aluminum-magnesium coated steel sheet with incision corrosion resistance wherein the hot-dipped zinc-aluminum-magnesium coated steel sheet comprises a steel sheet and a coating, **characterized in that**, the mass fractions of the chemical components in the coating are: 2% ~ 12% for aluminum, 1% ~ 4% for magnesium, 0.01% ~ 0.1% for calcium, and the rest being zinc and inevitable impurities; the mass fraction of aluminum is 2 to 3 times the mass fraction of magnesium; and the thickness of the coating is not less than 5‰ of the thickness of the steel sheet;
wherein the manufacturing method comprises:
obtaining a coating solution by using the chemical components of the coating of the hot-dipped zinc-aluminum-magnesium coated steel sheet ;
heating the coating solution to obtain a preheated coating solution with a temperature of the preheated coating solution being controlled to be not lower than a melting point of the coating solution and not higher than 500°C;
obtaining a steel sheet, and immersing the steel sheet in the preheated coating solution to obtain a coated steel sheet; and
cooling the coated steel sheet to obtain the hot-dipped zinc-aluminum-magnesium coated steel sheet;
wherein the cooling the coated steel sheet comprises:
when a temperature of the coated steel sheet is between a temperature of the coating bath and 360°C, the cooling is performed at a first cooling rate and the first cooling rate is controlled at: 0 < the first cooling rate ≤ 1°C/s; and
when the temperature of the coated steel sheet is between 360°C and 300°C, the cooling is performed at a second cooling rate and the second cooling rate is ≥ 5°C/s.

3. The manufacturing method of the hot-dipped zinc-aluminum-magnesium coated steel sheet according to claim 2, wherein, when the mass fraction of calcium is 0.01%, the mass fractions of magnesium and aluminum in the coating are controlled based on the thickness of the steel sheet, comprising:
when 0.5 mm ≤ the thickness of the steel sheet ≤ 2.5 mm, the mass fractions of chemical components in the coating are: 2% ~ 12% for aluminum, 1% ~ 4% for magnesium, and the rest being zinc and inevitable impurities;
when 2.5 mm < the thickness of the steel sheet ≤ 4 mm, the mass fractions of the chemical components in the coating are: 2.5% ~ 12% for aluminum, 1.2% ~ 4% for magnesium, and the rest being zinc and inevitable impurities;
when 4 mm < the thickness of the steel sheet ≤ 5 mm, the mass fractions of the chemical components in the coating are: 3.8% ~ 12% for aluminum, 1.8% ~ 4% for magnesium, and the rest being zinc and inevitable impurities; and
when 5 mm < the thickness of the steel sheet ≤ 6 mm, the mass fractions of the chemical components in the coating are: 5% ~ 12% for aluminum, 2.5% ~ 4% for magnesium, and the rest being zinc and inevitable impurities.

4. The manufacturing method of the hot-dipped zinc-aluminum-magnesium coated steel sheet according to claim 1 or 2, **characterized in that**, the steel sheet is preheated to a steel sheet preheating temperature before the immersion of the steel sheet in the coating solution for bathing, and a range of the steel sheet preheating temperature is the temperature of the preheated coating solution ± 10°C.

5. The manufacturing method of the hot-dipped zinc-aluminum-magnesium coated steel sheet according to claim 1 or 2, **characterized in that**, the steel sheet is preheated to a steel sheet preheating temperature before the immersion of the steel sheet in the coating solution for bathing, and the steel sheet preheating temperature is controlled based on the thickness of the steel sheet, comprising:
when 0.5 mm ≤ the thickness of the steel sheet ≤ 2 mm, the temperature of the preheated coating solution ≤ the steel sheet preheating temperature ≤ the temperature of the preheated coating solution + 10°C;
when 2 mm < the thickness of the steel sheet ≤ 4 mm, the temperature of the preheated coating solution - 5°C ≤ the steel sheet preheating temperature ≤ the temperature of the preheated coating solution; and
when 4 mm < the thickness of the steel sheet ≤ 6 mm, the temperature of the preheated coating solution - 10°C ≤ the steel sheet preheating temperature ≤ the temperature of the preheated coating solution - 5°C.

6. The manufacturing method of the hot-dipped zinc-aluminum-magnesium coated steel sheet according to claim 1 or 2, **characterized in that**, the obtaining the steel sheet comprises obtaining the steel sheet with a surface roughness Ra of 1 µm ~ 2 µm.

## Patentansprüche

1. Herstellungsverfahren eines feuerverzinkten Zink-Aluminium-Magnesium-beschichteten Stahlblechs mit Einschnittkorrosionsbeständigkeit,
**dadurch gekennzeichnet, dass** das feuerverzinkte Zink-Aluminium-Magnesium-beschichtete Stahlblech ein Stahlblech und eine Beschichtung umfasst,
wobei die Massenanteile der chemischen Komponenten in der Beschichtung Folgende sind: 2 % bis 12 % für Aluminium, 1 % bis 4 % für Magnesium, wobei der Rest aus Zink und unvermeidbaren Verunreinigungen besteht; und der Massenanteil von Aluminium beträgt das 2- bis 3-fache des Massenanteils von Magnesium; und
eine Dicke der Beschichtung nicht weniger als 5 % der Dicke des Stahlblechs ist;
wobei die Dicke des Stahlblechs im Bereich von 0,5 mm bis 6 mm liegt;
wobei die Massenanteile von Magnesium und Aluminium in der Beschichtung basierend auf der Dicke des Stahlblechs gesteuert werden, umfassend:
Wenn 0,5 mm ≤ die Dicke des Stahlblechs ≤ 2 mm, betragen die Massenanteile der chemischen Komponenten in der Beschichtung: 2 % bis 12 % für Aluminium, 1 % bis 4 % für Magnesium, wobei der Rest aus Zink und unvermeidbaren Verunreinigungen besteht;
Wenn 2 mm ≤ die Dicke des Stahlblechs ≤ 4 mm, betragen die Massenanteile der chemischen Komponenten in der Beschichtung: 3 % bis 12 % für Aluminium, 1,5 % bis 4 % für Magnesium, wobei der Rest aus Zink und unvermeidbaren Verunreinigungen besteht;
Wenn 4 mm ≤ die Dicke des Stahlblechs ≤ 5 mm, betragen die Massenanteile der chemischen Komponenten in der Beschichtung: 4 % bis 12 % von Aluminium, 2 % bis 4 % von Magnesium, wobei der Rest aus Zink und unvermeidbaren Verunreinigungen besteht; und
Wenn 5 mm ≤ die Dicke des Stahlblechs ≤ 6 mm, betragen die Massenanteile der chemischen Komponenten in der Beschichtung: 6 % bis 12 % für Aluminium, 3 % bis 4 % für Magnesium, wobei der Rest aus Zink und unvermeidbaren Verunreinigungen besteht;
wobei das Herstellungsverfahren Folgendes umfasst:
Herstellen einer Beschichtungslösung durch Verwenden der chemischen Komponenten der Beschichtung des feuerverzinkten Zink-Aluminium-Magnesium-beschichteten Stahlblechs;
Erwärmen der Beschichtungslösung, um eine vorgewärmte Beschichtungslösung zu erhalten, wobei die Temperatur der vorgewärmten Beschichtungslösung so geregelt wird, dass sie nicht unter dem Schmelzpunkt der Beschichtungslösung und nicht über 500 °C liegt;
Bereitstellen eines Stahlblechs und Eintauchen des Stahlblechs in die vorgewärmte Beschichtungslösung, um ein beschichtetes Stahlblech zu erhalten; und
Abkühlen des beschichteten Stahlblechs, um das feuerverzinkte Zink-Aluminium-Magnesium-beschichtete Stahlblech zu erhalten;
wobei das Abkühlen des beschichteten Stahlblechs Folgendes umfasst:
wenn die Temperatur des beschichteten Stahlblechs zwischen der Temperatur des Beschichtungsbads und 360 °C liegt, wird das Abkühlen mit einer ersten Abkühlrate durchgeführt, wobei die erste Abkühlrate wie folgt gesteuert wird: 0 ≤ die erste Abkühlrate ≤ 1 °C/s; und
wenn die Temperatur des beschichteten Stahlblechs zwischen 360 °C und 300 °C liegt, wird die Abkühlung mit einer zweiten Abkühlrate durchgeführt, und die zweite Abkühlrate beträgt ≥ 5 °C/s.

2. Herstellungsverfahren eines feuerverzinkten Zink-Aluminium-Magnesium-beschichteten Stahlblechs mit Einschnittkorrosionsbeständigkeit,
wobei das feuerverzinkte Zink-Aluminium-Magnesium beschichtete Stahlblech ein Stahlblech und eine Beschichtung umfasst, **dadurch gekennzeichnet, dass** die Massenanteile der chemischen Komponenten in der Beschichtung Folgende sind: 2 % bis 12 % für Aluminium, 1 % bis 4 % für Magnesium, 0,01 % bis 0,1 % für Kalzium, wobei der Rest aus Zink und unvermeidbaren Verunreinigungen besteht; der Massenanteil von Aluminium beträgt das 2- bis 3-fache des Massenanteils von Magnesium; und die Dicke der Beschichtung nicht weniger als 5 % der Dicke des Stahlblechs ist;
wobei das Herstellungsverfahren Folgendes umfasst:
Herstellen einer Beschichtungslösung durch Verwenden der chemischen Komponenten der Beschichtung des feuerverzinkten Zink-Aluminium-Magnesium-beschichteten Stahlblechs;
Erwärmen der Beschichtungslösung, um eine vorgewärmte Beschichtungslösung zu erhalten, wobei die Temperatur der vorgewärmten Beschichtungslösung so geregelt wird, dass sie nicht unter dem Schmelzpunkt der Beschichtungslösung und nicht über 500 °C liegt;
Bereitstellen eines Stahlblechs und Eintauchen des Stahlblechs in die vorgewärmte Beschichtungslösung, um ein beschichtetes Stahlblech zu erhalten; und
Abkühlen des beschichteten Stahlblechs, um das feuerverzinkte Zink-Aluminium-Magnesium-beschichtete Stahlblech zu erhalten;
wobei das Abkühlen des beschichteten Stahlblechs Folgendes umfasst:
wenn die Temperatur des beschichteten Stahlblechs zwischen der Temperatur des Beschichtungsbads und 360 °C liegt, wird das Abkühlen mit einer ersten Abkühlrate durchgeführt, wobei die erste Abkühlrate wie folgt gesteuert wird: 0 ≤ die erste Abkühlrate ≤ 1 °C/s; und
wenn die Temperatur des beschichteten Stahlblechs zwischen 360 °C und 300 °C liegt, wird die Abkühlung mit einer zweiten Abkühlrate durchgeführt, und die zweite Abkühlrate beträgt ≥ 5 °C/s.

3. Herstellungsverfahren des feuerverzinkten Zink-Aluminium-Magnesium beschichteten Stahlblechs nach Anspruch 2, wobei bei einem Massenanteil von Kalzium von 0,01 % die Massenanteile von Magnesium und Aluminium in der Beschichtung basierend auf der Dicke des Stahlblechs gesteuert werden, umfassend:
Wenn 0,5 mm ≤ die Dicke des Stahlblechs ≤ 2,5 mm, betragen die Massenanteile von chemischen Komponenten in der Beschichtung: 2 % bis 12 % für Aluminium, 1 % bis 4 % für Magnesium, wobei der Rest aus Zink und unvermeidbaren Verunreinigungen besteht;
Wenn 2,5 mm ≤ die Dicke des Stahlblechs ≤ 4 mm, betragen die Massenanteile der chemischen Komponenten in der Beschichtung: 2,5 % bis 12 % für Aluminium, 1,2 % bis 4 % für Magnesium, wobei der Rest aus Zink und unvermeidbaren Verunreinigungen besteht;
Wenn 4 mm ≤ die Dicke des Stahlblechs ≤ 5 mm, betragen die Massenanteile der chemischen Komponenten in der Beschichtung: 3,8 % bis 12 % für Aluminium, 1,8 % bis 4 % für Magnesium, wobei der Rest aus Zink und unvermeidbaren Verunreinigungen besteht; und
Wenn 5 mm ≤ die Dicke des Stahlblechs ≤ 6 mm, betragen die Massenanteile der chemischen Komponenten in der Beschichtung: 5 % bis 12 % für Aluminium, 2,5 % bis 4 % für Magnesium, wobei der Rest aus Zink und unvermeidbaren Verunreinigungen besteht.

4. Herstellungsverfahren des feuerverzinkten Zink-Aluminium-Magnesium beschichteten Stahlblechs nach Anspruch 1 oder 2, **dadurch gekennzeichnet, dass** das Stahlblech vor dem Eintauchen in die Beschichtungslösung auf eine Vorwärmtemperatur für das Stahlblech vorgewärmt wird und der Bereich der Vorwärmtemperatur für das Stahlblech der Temperatur der vorgewärmten Beschichtungslösung ± 10 °C entspricht.

5. Herstellungsverfahren des feuerverzinkten Zink-Aluminium-Magnesium beschichteten Stahlblechs nach Anspruch 1 oder 2, **dadurch gekennzeichnet, dass** das Stahlblech vor dem Eintauchen in die Beschichtungslösung auf eine Vorwärmtemperatur für das Stahlblech vorgewärmt wird und die Vorwärmtemperatur für das Stahlblech basierend auf der Dicke des Stahlblechs geregelt wird, umfassend:
Wenn 0,5 mm ≤ Dicke des Stahlblechs ≤ 2 mm, die Temperatur der vorgewärmten Beschichtungslösung ≤ Vorwärmtemperatur des Stahlblechs ≤ Temperatur der vorgewärmten Beschichtungslösung + 10 °C;
Wenn 2 mm ≤ die Dicke des Stahlblechs ≤ 4 mm, die Temperatur der vorgewärmten Beschichtungslösung - 5 °C ≤ die Vorwärmtemperatur des Stahlblechs ≤ die Temperatur der vorgewärmten Beschichtungslösung; und
Wenn 4 mm ≤ die Dicke des Stahlblechs ≤ 6 mm, die Temperatur der vorgewärmten Beschichtungslösung - 10 °C < die Vorwärmtemperatur des Stahlblechs ≤ die Temperatur der vorgewärmten Beschichtungslösung - 5 °C.

6. Herstellungsverfahren des feuerverzinkten Zink-Aluminium-Magnesium beschichteten Stahlblechs nach Anspruch 1 oder 2, **dadurch gekennzeichnet, dass** das Erhalten des Stahlblechs das Erhalten eines Stahlblechs mit einer Oberflächenrauheit Ra von 1 µm bis 2 µm umfasst.

## Revendications

1. Procédé de fabrication d'une tôle d'acier revêtue de zinc-aluminium-magnésium trempée à chaud avec une résistance à la corrosion par incision,
**caractérisé en ce que** la tôle d'acier revêtue de zinc-aluminium-magnésium trempée à chaud comprend une tôle d'acier et un revêtement,
des fractions massiques des composants chimiques dans le revêtement sont comme suit : 2% ~ 12% pour l'aluminium, 1% - 4% pour le magnésium, et le reste étant du zinc et des impuretés inévitables ; et la fraction massique d'aluminium est de 2 à 3 fois la fraction massique de magnésium ; et
une épaisseur du revêtement n'est pas inférieure à 5 ‰ d'une épaisseur de la tôle d'acier ;
dans lequel, l'épaisseur de la tôle d'acier va de 0,5 mm à 6 mm ;
dans lequel les fractions massiques de magnésium et d'aluminium dans le revêtement sont contrôlées sur la base de l'épaisseur de la tôle d'acier, comprenant :
lorsque 0,5 mm ≤ l'épaisseur de la tôle d'acier ≤ 2 mm, les fractions massiques des composants chimiques dans le revêtement sont comme suit : 2% - 12% pour l'aluminium, 1% - 4% pour le magnésium, et le reste étant du zinc et des impuretés inévitables ;
lorsque 2 mm < l'épaisseur de la tôle d'acier ≤ 4 mm, les fractions massiques des composants chimiques dans le revêtement sont comme suit : 3% - 12% pour l'aluminium, 1,5% - 4% pour le magnésium, et le reste étant du zinc et des impuretés inévitables ;
lorsque 4 mm < l'épaisseur de la tôle d'acier ≤ 5 mm, les fractions massiques des composants chimiques dans le revêtement sont comme suit : 4% - 12% d'aluminium, 2% - 4% de magnésium, et le reste étant du zinc et des impuretés inévitables ; et
lorsque 5 mm < l'épaisseur de la tôle d'acier ≤ 6 mm, les fractions massiques des composants chimiques dans le revêtement sont comme suit : 6% - 12% pour l'aluminium, 3% - 4% pour le magnésium, et le reste étant du zinc et des impuretés inévitables ;
dans lequel le procédé de fabrication comprend :
l'obtention d'une solution de revêtement en utilisant les composants chimiques du revêtement de la tôle d'acier revêtue de zinc-aluminium-magnésium trempée à chaud ;
le chauffage de la solution de revêtement pour obtenir une solution de revêtement préchauffée avec une température de la solution de revêtement préchauffée régulée de façon à ne pas être inférieure à un point de fusion de la solution de revêtement et pas supérieure à 500°C ;
l'obtention d'une tôle d'acier, et l'immersion de la tôle d'acier dans la solution de revêtement préchauffée pour obtenir une tôle d'acier revêtue ; et
le refroidissement de la tôle d'acier revêtue pour obtenir la tôle d'acier revêtue de zinc-aluminium-magnésium trempée à chaud ;
dans lequel le refroidissement de la tôle d'acier revêtue comprend :
lorsqu'une température de la tôle d'acier revêtue est entre une température du bain de revêtement et 360°C, le refroidissement est effectué selon une première vitesse de refroidissement et la première vitesse de refroidissement est régulée à : 0 < la première vitesse de refroidissement ≤ 1°C/s ; et
lorsque la température de la tôle d'acier revêtue est entre 360°C et 300°C, le refroidissement est effectué à une deuxième vitesse de refroidissement et la deuxième vitesse de refroidissement est ≥ 5°C/s.

2. Procédé de fabrication d'une tôle d'acier revêtue de zinc-aluminium-magnésium trempée à chaud avec une résistance à la corrosion par incision,
dans lequel la tôle d'acier revêtue de zinc-aluminium-magnésium trempée à chaud comprend une tôle d'acier et un revêtement, **caractérisé en ce que** les fractions massiques des composants chimiques dans le revêtement sont comme suit : 2% ~ 12% pour l'aluminium, 1% - 4% pour le magnésium, 0,01% - 0,1% pour le calcium, et le reste étant du zinc et des impuretés inévitables ; la fraction massique d'aluminium est de 2 à 3 fois la fraction massique de magnésium ; et l'épaisseur du revêtement n'est pas inférieure à 5% de l'épaisseur de la tôle d'acier ;
dans lequel le procédé de fabrication comprend :
l'obtention d'une solution de revêtement en utilisant les composants chimiques du revêtement de la tôle d'acier revêtue de zinc-aluminium-magnésium trempée à chaud ;
le chauffage de la solution de revêtement pour obtenir une solution de revêtement préchauffée avec une température de la solution de revêtement préchauffée régulée de façon à ne pas être inférieure à un point de fusion de la solution de revêtement et pas supérieure à 500°C ;
l'obtention d'une tôle d'acier, et l'immersion de la tôle d'acier dans la solution de revêtement préchauffée pour obtenir une tôle d'acier revêtue ; et
le refroidissement de la tôle d'acier revêtue pour obtenir la tôle d'acier revêtue de zinc-aluminium-magnésium trempée à chaud ;
dans lequel le refroidissement de la tôle d'acier revêtue comprend :
lorsqu'une température de la tôle d'acier revêtue est entre une température du bain de revêtement et 360°C, le refroidissement est effectué selon une première vitesse de refroidissement et la première vitesse de refroidissement est régulée à : 0 < la première vitesse de refroidissement ≤ 1°C/s ; et
lorsque la température de la tôle d'acier revêtue est entre 360°C et 300°C, le refroidissement est effectué à une deuxième vitesse de refroidissement et la deuxième vitesse de refroidissement est ≥ 5°C/s.

3. Procédé de fabrication de la tôle d'acier revêtue de zinc-aluminium-magnésium trempée à chaud selon la revendication 2, dans lequel, lorsque la fraction massique de calcium est de 0,01%, les fractions massiques de magnésium et d'aluminium dans le revêtement sont contrôlées sur la base de l'épaisseur de la tôle d'acier, comprenant :
lorsque 0,5 mm ≤ l'épaisseur de la tôle d'acier ≤ 2,5 mm, les fractions massiques des composants chimiques dans le revêtement sont comme suit : 2% - 12% pour l'aluminium, 1% - 4% pour le magnésium, et le reste étant du zinc et des impuretés inévitables ;
lorsque 2,5 mm < l'épaisseur de la tôle d'acier ≤ 4 mm, les fractions massiques des composants chimiques dans le revêtement sont comme suit : 2,5% ~ 12% pour l'aluminium, 1,2% - 4% pour le magnésium, et le reste étant du zinc et des impuretés inévitables ;
lorsque 4 mm < l'épaisseur de la tôle d'acier ≤ 5 mm, les fractions massiques des composants chimiques dans le revêtement sont comme suit : 3,8% - 12% pour l'aluminium, 1,8% - 4% pour le magnésium, et le reste étant du zinc et des impuretés inévitables ; et
lorsque 5 mm < l'épaisseur de la tôle d'acier ≤ 6 mm, les fractions massiques des composants chimiques dans le revêtement sont comme suit : 5% - 12% pour l'aluminium, 2,5% - 4% pour le magnésium, et le reste étant du zinc et des impuretés inévitables.

4. Procédé de fabrication de la tôle d'acier revêtue de zinc-aluminium-magnésium trempée à chaud selon la revendication 1 ou 2, **caractérisé en ce que**, la tôle d'acier est préchauffée à une température de préchauffage de tôle d'acier avant l'immersion de la tôle d'acier dans la solution de revêtement pour le bain, et une plage de la température de préchauffage de tôle d'acier est la température de la solution de revêtement préchauffée ± 10°C.

5. Procédé de fabrication de la tôle d'acier revêtue de zinc-aluminium-magnésium trempée à chaud selon la revendication 1 ou 2, **caractérisé en ce que**, la tôle d'acier est préchauffée à une température de préchauffage de tôle d'acier avant l'immersion de la tôle d'acier dans la solution de revêtement pour le bain, et la température de préchauffage de tôle d'acier est régulée sur la base de l'épaisseur de la tôle d'acier, comprenant :
lorsque 0,5 mm ≤ l'épaisseur de la tôle d'acier ≤ 2 mm, la température de la solution de revêtement préchauffée ≤ la température de préchauffage de tôle d'acier ≤ la température de la solution de revêtement préchauffée + 10°C ;
lorsque 2 mm < l'épaisseur de la tôle d'acier ≤ 4 mm, la température de la solution de revêtement préchauffée - 5°C ≤ la température de préchauffage de tôle d'acier ≤ la température de la solution de revêtement préchauffée ; et
lorsque 4 mm < l'épaisseur de la tôle d'acier ≤ 6 mm, la température de la solution de revêtement préchauffée - 10°C ≤ la température de préchauffage de tôle d'acier ≤ la température de la solution de revêtement préchauffée - 5°C.

6. Procédé de fabrication de la tôle d'acier revêtue de zinc-aluminium-magnésium trempée à chaud selon la revendication 1 ou 2, **caractérisé en ce que**, l'obtention de la tôle d'acier comprend l'obtention de la tôle d'acier avec une rugosité de surface Ra de 1 µm ~ 2 µm.
